

## UNITED STATES PATENT OFFICE

WILLIAM G. LEAMON, OF NEWARK, OHIO

## ART OF TREATING OILS

No Drawing. Application filed February 24, 1923, Serial No. 621,076. Renewed December 28, 1925.

This invention relates to art of treating more or less obscure as to exact chemical oils; and more particularly to the treatment of hydrocarbon oils such as petroleum, petroleum distillates and residue, in the manufacture of valuable commercial products.

The invention is concerned especially with what may be broadly termed a modifying treatment of oils with the aid of a catalytic material which may function either as an agent for assisting conversion of relatively heavy oils into lighter oils of lower boiling points, or chiefly as a polymerizing or condensing agent in such manner as to enable removal of undesirable constituents from a given oil without necessarily effecting conversion in the sense of cracking. In some cases the catalytic material may function in both ways. It is to be understood that the term catalyst or catalytic agent or material is used herein in a broad sense to include a wide range of substances known under that head or under the head of contact, condensing, carrying, accelerating and promoting agents.

While the invention is considered to be of broad scope in its general applicability to oils of widely divergent characteristics and for the manufacture of various products, its most important commercial application at the present time is the treatment of relatively light petroleum distillates, having specific gravities of from about .730 to .830, and distillation ranges lying between about 100° and 600° F., particularly motor fuels, gasolines, and other motor fuels of that general type, as well as kerosenes, for increasing stability thereof and otherwise improving the same. Accordingly this phase of the matter will be more especially emphasized and described in detail in the following specification.

It is common knowledge that commercial gasolines or other motor fuels heretofore available are ordinarily unstable, especially those made by cracking processes; that is, they undergo substantial changes in composition in a comparatively short time under storage conditions, these changes being highly undesirable and prejudicial to attainment of best results in utilizing the fuel. While

character, these changes are known to result in the formation of compounds in the gasoline or other motor fuel which, upon evaporation of the motor fuel, manifest themselves in the form of a more or less gummy or resinous residue. In the case of some motor fuels, this resinous or gummy formation occurs to such an extent that, even without evaporation, an insoluble residue of said material is deposited upon the bottom of containers in which the motor fuel is stored. In all cases, however, whether deposition of the gummy material occurs before evaporation or not, the necessary potential constituents thereof are present in ordinary commercial motor fuels, a fact which can be shown by test soon after final distillation. This tendency is usually more pronounced in the case of motor fuels obtained from the various cracking processes, which fuels are characterized by a substantial content of unsaturates. However, the extent to which the undesirable gummy or resinous compounds are formed does not appear to bear any simple or direct relation to the quantity of unsaturates present in a given motor fuel; and this formation of gummy or resinous compounds, or instability, is characteristic of many commercial straight-run gasolines as well as gasolines produced by cracking.

It is generally believed that the instability above referred to is due at least largely to polymerization of certain constituents invariably present in gasolines or other motor fuels as commercially produced heretofore, this polymerization beginning very soon after distillation and progressing usually rather slowly at a rate depending upon the character of the particular motor fuel in question and the conditions of its storage. Sometimes part of the final polymerization products separate out, but the greater part remain in solution. The practical effect of this polymerization is that upon evaporation the resultant gummy polymers which then separate foul the carburetors and valves of internal combustion engines in which the fuel is used, causes excessive carbonizing, and are otherwise seriously objectionable.

The foregoing objections to commercial motor fuels heretofore available have been recognized for a long time and there have been various proposals to obviate them; but so far as I am aware, none of these prior proposals has proved successful.

It is a specific object of the present invention to provide a simple and effective method for stabilizing gasolines and other motor fuels and to produce a motor fuel that does in fact remain stable for long periods. Another object of the invention is to provide a method that is not only simple and effective but is also economical and, in particular, a method by which gasolines or other motor fuels relatively very high in unsaturates can be stabilized without necessarily reducing their content of unsaturates to any substantial extent. Further objects of the invention are in general to enable treatment of any oil product, whether for conversion, stabilization, or for otherwise improving the same, with the aid of a contact or catalyzing agent, particularly a catalytic metallic halide, brought into contact with the oil in a much more intimate and effective manner than as been possible heretofore.

With these and other objects in view, the invention comprises the novel process which will be hereinafter more fully described in connection with typical illustrative embodiments thereof and will then be more particularly pointed out in the claims.

In order to explain more fully the principles underlying the invention, the stabilization of a motor fuel or gasoline in accordance with the invention will be more particularly referred to and described in detail as illustrating a practical application of the invention in one of its most advantageous forms. Described in general terms, the method of treatment is one which greatly expedites the formation of the polymers constituting the gummy or resinous products that are eventually formed after ordinary gasoline has stood for a greater or less period of time after distillation. It is possible by the treatment to carry this polymerization to a conclusion within a space of time extremely short as compared to the normally rather slow progress of polymerization, and at the same time to effect this result at substantially room temperature without otherwise perceptibly affecting the constitution of the gasoline undergoing treatment. It is not to be understood, however, that the invention in its broad aspects is restricted to the use of such low temperature. The polymerizing action having been thus expedited and completed, separation of the gummy polymers from the motor fuel can be readily effected, and the motor fuel is then stable.

In practicing the invention for stabilizing gasoline the polymerizing agent employed

may be any one of various catalytic or contact materials found suitable for the purpose; but in general the action of catalytic metallic halides has been found most effective, anhydrous aluminum chlorid being especially well adapted for use in practice. Anhydrous ferric chlorid also gives good results as does also anhydrous zinc chlorid.

In order to obtain effective action of the polymerizing agent, it is essential that it be brought into extremely intimate reacting contact with all parts of the motor fuel to be treated. In the best mode of practicing the invention, this is accomplished by treating the motor fuel with a solution of the polymerizing agent in a solvent that is miscible with or soluble in the motor fuel to such an extent as to ensure distribution of said agent therethrough and substantially molecular contact with all parts thereof. This mode of procedure enormously increases the velocity of the polymerizing reaction by which gummy constituents are formed. Thus, by dissolving aluminum chlorid in a suitable solvent that is miscible with the gasoline or other motor fuel to be treated, and mixing this solution with the gasoline at ordinary room temperatures, it is found that apparently complete polymerization of the polymerizable constituents present in the untreated gasoline is effected substantially at once, that is, within a very few minutes, or at most a few hours. Some of the products of polymerization separate out in insoluble form very soon after the addition of the aluminum chlorid solution, and with them also separates a large proportion, usually nearly all, of the aluminum chlorid that was used. In most cases, a large part of the products of polymerization remain dissolved in the gasoline, together with a minute proportion of the aluminum chlorid. After treatment with the aluminum chlorid solution, the gasoline may or may not be filtered to remove the initial precipitate of polymers and aluminum chlorid, and is then usually distilled to effect separation of the polymers still remaining in the gasoline. The resultant distillate is a gasoline of notably superior characteristics; and when the process is carried out under the best conditions, said distillate is a truly stable gasoline in the sense that even after standing for a long period, say three months or more, it shows substantially no content of gummy or resinous matter when subjected to tests for this characteristic. The odor of the gasoline is also generally improved perceptibly, as is also its color, a water white product being obtainable by this method from a yellow gasoline. The constitution of the gasoline as regards its content of unsaturates or freedom therefrom, is apparently not altered substantially when the

process is carried out in the manner described.

In a specific instance, let it be assumed that the motor fuel to be stabilized is a product obtained by cracking, and is of a type containing up to as much as 20 to 40 per cent of unsaturates as determined by the fuming sulfuric acid test, said type having a specific gravity ranging from .730 to .780 and a distillation range lying between about 100° to 460° or 475° F. as outside limits. In treating this or any other type of motor fuel in accordance with the process of the invention, it is advisable first to determine how much anhydrous aluminum chlorid ( $Al_2Cl_6$ ) is required to take up or otherwise render inactive any moisture present as such or as  $H_2O$  held either chemically or in some other analogous manner by the hydrocarbons of the motor fuel; since, in order to obtain the desired stabilizing results, the presence of some anhydrous aluminum chlorid is essential, and hence an excess of aluminum chlorid should be employed over what is converted into  $Al_2Cl_6 \cdot 12H_2O$  in dehydrating the gasoline. Accordingly, a sample of the motor fuel is titrated with a standard solution of anhydrous aluminum chlorid ( $Al_2Cl_6$ ) in sulfuric ether (ethyl ether) until the point is reached where the next drop of standard solution produces a permanently reddish coloration of the titration mixture. The end point is sharp, and when titration has been properly performed, the reddish coloration of the mixture at the end point may be instantly dissipated merely by breathing upon the mixture, the slight amount of moisture thus introduced being sufficient to destroy the red color. From the results of this titration it is a simple matter to compute the amount of anhydrous aluminum chlorid necessary to combine with the moisture in the motor fuel, which quite commonly amounts to around 0.05 per cent. Only a slight excess over this amount need be used in the stabilizing treatment. With a motor fuel such as that above assumed, it is found that the employment of from 5 to 6 ounces of dissolved anhydrous aluminum chlorid per each barrel of 42 gallons, is amply sufficient both to allow for dehydration and to ensure stabilization being effected. This amounts to slightly more than one-tenth of one per cent on the weight of gasoline treated, and is fairly representative of average practice in carrying on my invention commercially. In general it is unnecessary to employ more than a fraction of one per cent, and usually only a minor fraction. The ability to operate with such small percentages of catalyst indicates how enormously active it is when employed in accordance with the principles of my invention. It appears probable that this is due in large measure to obtaining molecular contact, or something analogous thereto, between the aluminum chlorid and

the gasoline treated, through the distributing action of the solvent or carrier, although it is also possibly due to formation of complex combinations between the solvent and the gums of gum-forming constituents. The aluminum chlorid is not soluble in the gasoline alone to a useful extent.

Where the moisture content of the motor fuel is considerable, as it may be in some cases, it may be desirable from the standpoint of economy first to filter it through, or otherwise to treat it with, a cheaper dehydrating agent such as caustic lime or calcium chlorid to reduce the moisture content as far as is practicable by such methods before treating with anhydrous aluminum chlorid.

The required amount of anhydrous aluminum chlorid having been computed from the test titration, this amount is added to the gasoline or other motor fuel in the form of a solution in a suitable solvent of aluminum chlorid, and most desirably in a solvent that is miscible with or soluble in said gasoline or any other motor fuel. Any one of various solvents can be employed, and it is to be understood that the invention is not limited in this respect. It has been found, however, that alcohol ( $C_2H_5OH$ ) is not a suitable solvent to employ with aluminum chlorid in practicing the invention, and accordingly alcohol is not to be understood as included among those recommended herein. Uniform distribution of the reagent through the motor fuel is attained by stirring or otherwise agitating, if necessary. In practice sulfuric ether is an excellent solvent to use, since it dissolves anhydrous aluminum chlorid very readily up to as much as from two to two and one-half times its own weight at room temperature, and is also readily miscible with or soluble in the motor fuel in the proportions necessary to employ it in practicing the invention. Moreover, the finished motor fuel obtained when an ether solution of aluminum chlorid is used in carrying out the novel method is of exceptionally good color and stability. Mononitrobenzene is also a good solvent for the purpose. Where ether is employed, it is good practice to use a solution containing equal parts by weight of anhydrous aluminum chlorid and ether. The solution may be added to and mixed with the motor fuel at ordinary room temperature, no heating being required to bring about the polymerizing action which takes place with great rapidity and may be practically complete within a few minutes or at most within a few hours after addition of the ether solution of the polymerizing agent. Immediately after the ether solution has been added, a precipitate begins to separate out, and in order to allow ample time to complete this separation it is good practice to allow the treated motor fuel to stand for a period that may range from one hour to twenty-four hours. The precipitate

comes out and settles in the form of more or less irregularly shaped gummy particles that are easily separated from the liquid either by filtration or by decantation. Separation of the precipitate at this stage is optional although in general it is to be recommended if the precipitate is at all large. An examination of the precipitate shows that it consists largely of gummy polymers together with nearly all of the aluminum chlorid originally introduced into the motor fuel. The clear solution contains, however, a large proportion of the formed polymers that remain dissolved and do not separate at this stage, together with a trace of aluminum chlorid. It is sometimes desirable also, before separating the precipitate, to eliminate even the residual trace of aluminum chlorid from the motor fuel by treating the same with a suitable precipitating agent for aluminum as, for example, by agitating with a small quantity of dry sodium bicarbonate, or with a small amount of an alcoholic solution of caustic soda or potash. In this case, the motor fuel, after separation of insoluble matter by filtration or decantation, contains substantially no trace of aluminum chlorid, and is also substantially neutral in reaction.

In the specific example here assumed, the treated motor fuel is next re-distilled to separate therefrom the polymerized constituents that still remain in solution as result of the treatment with aluminum chlorid. This distillation may be effected in the usual manner and requires no special precautions other than those employed in ordinary practice. The distillate is a finished motor fuel which is stable, sweet in odor and of excellent color, as already pointed out. The content of unsaturates is substantially the same as in the original motor fuel, about 30 per cent in a typical instance. This is a highly advantageous feature of the process, since a motor fuel containing unsaturates, when stabilized in accordance with the invention, gives better mileage and greater power than a motor fuel that contains no unsaturates. Furthermore, it is to be especially noted that this high grade motor fuel is obtainable without the large refinery loss resulting from the commonly employed sulfuric acid treatment for removal of unsaturates.

In the case of motor fuels that are high in unsaturates, such as that whose treatment has been described in detail above, it is generally the best practice always to redistill after treatment with the solution of anhydrous aluminum chlorid. However, in the case of straight run gasolines, for example, which are commonly obtained by topping crude petroleum and which are often practically free from unsaturates, the benefits of the invention can be realized to a very substantial extent even where there is no redistillation after treatment with the solution

of anhydrous aluminum chlorid; although even straight-run gasolines should be redistilled to attain the best results. Many straight-run gasolines, however, contain such comparatively small amounts of constituents polymerizable to gums that they are generally quite acceptable commercially even though not stable, strictly speaking. In the case of such gasolines, treatment with a solution of anhydrous aluminum chlorid or other suitable polymerizing agent has the effect of polymerizing whatever polymerizable constituents are present, but the polymers do not separate upon standing at ordinary temperatures to so great an extent as in the case of a motor fuel high in unsaturates. There is usually some separation of polymers, together with practically all of the aluminum chlorid; but a large proportion of them remains dissolved in the motor fuel. Nevertheless the improvement in odor and color of the motor fuel, even without redistillation after treatment, is so marked as to render it of much greater commercial value. In such cases, after separation of such solid matter as may precipitate upon standing for from one to twenty-four hours in the cold, but without re-distilling, the treated motor fuel can be marketed as a finished product of a quality superior to untreated straight-run gasolines. As before stated, however, gasoline so treated, but not distilled, is not stable because it still contains dissolved gummy polymers which are deposited upon evaporation of the gasoline.

From the foregoing it is apparent that, while redistillation after treatment with aluminum chlorid is an important feature of the invention in certain of its advantageous embodiments, it is not to be regarded as an indispensable step of the novel process in all cases.

In the manufacture of gasolines and like motor fuels by topping crudes or by cracking, it is common practice to obtain from the topping still, cracking still, cracking tubes, or other suitable source, a crude motor fuel which is then re-run to improve its boiling range by eliminating the heavy ends contained therein. Where this is customary, the treatment with a solution of aluminum chlorid in accordance with the invention may most advantageously be applied to the crude distillate before it is re-run or re-distilled. This involves no change in the regular practice other than the addition of the aluminum chlorid solution and mixing thereof with the crude distillate by stirring or agitation, if desired, together with optional removal of the gummy precipitate that thereafter separates upon standing; all of which is readily interposed between the two usual steps of obtaining the crude motor fuel and re-running. It is to be understood, therefore that the process of the invention may comprise, in

one of its advantageous practical embodiments, the complete series of steps above set forth, beginning with the obtaining of a crude gasoline or the like by straight-run distillation of, or by cracking, petroleum or other relatively heavy oil material.

5 A stable petroleum distillate obtained in accordance with the process of the invention is believed to be a broadly novel product in the art and distinguishable from motor fuels heretofore known. In particular, a stable motor fuel containing unsaturates, especially a substantial or high percentage thereof, say 10 per cent or more, is a novel product 10 notably superior to motor fuels heretofore available.

In order to make clear the distinction between a truly stable motor fuel as obtainable by the practice of the invention, and the 20 unstable motor fuels heretofore exclusively available, it may be well to outline briefly a common test for stability as employed in regular practice. The tendency of a motor fuel to change in constitution or composition is manifested, as already pointed out, by 25 gummy substances developed therein and sometimes eventually deposited therefrom in insoluble form after the lapse of a period of time that varies with different motor fuels.

30 Deposit of these gummy substances may be hastened by evaporation, and the amount deposited will depend to a great extent upon the conditions of the evaporation. Accordingly, the amount of gummy substance deposited by evaporation of a given volume 35 of motor fuel under standard conditions is generally taken to indicate the degree of stability or instability of the motor fuel.

An investigation of the best motor fuels 40 heretofore known in the art shows that slow evaporation of 50 cubic centimeters in an open dish gently heated invariably yields a residue of at least three to five milligrams, and a motor fuel leaving so small a 45 gummy deposit as this is very exceptional. As a rule the amount is larger than this and it commonly ranges anywhere from 20 to 50 mgs. In contrast to this, a motor fuel treated with a solution of aluminum chlorid 50 and then re-distilled, as herein disclosed, when subjected to the evaporation test mentioned, leaves at the most a substantially smaller residue than three milligrams upon evaporation of 50 cubic centimeters thereof; 55 and as a rule the residue does not exceed two milligrams at the outside, being more commonly as little as 0.5 milligram.

The principles of the invention may also be 60 extended to the stabilizing or improvement generally of other petroleum products, such as lubricating oils, paraffine, and the like, which are not necessarily distillates, by treatment with a solution of a catalytic metallic halide, especially anhydrous aluminum 65 chlorid, in a suitable solvent miscible with the

product to be improved. The process may also be extended with advantage to conversion of heavy oils into lighter under cracking conditions, the important point here also being that the anhydrous aluminum chlorid or other suitable assisting agent be distributed throughout the mass of oil by means of a solvent differing from but miscible with the oil, whereby substantially molecular or analogous contact between the oil and the catalytic agent or assistant is attained, and the efficiency of the converting action is enhanced.

The principles of the invention may be extended further to cases where production of 70 polymerized materials from a hydrocarbon oil or distillate is a primary object rather than stabilization or other improvement of the hydrocarbon oil itself. The polymers obtained in treating gasoline or the like in accordance with the present invention have 75 value in the manufacture of lubricants, resins, and other products; and the production of such polymers is therefore an important phase 80 of the invention. In this particular aspect 85 of the invention also, the novel process is especially applicable to cracked mineral oil distillates since these are most likely to yield polymers in commercial quantities upon 90 treatment.

95 It is to be understood that the invention is not limited to the particular details hereinabove set forth by way of illustrative example, but that it is susceptible of being varied considerably in practice without departing from the underlying principles involved.

100 What I claim is:

105 1. The process of improving a hydrocarbon motor fuel which comprises commingling therewith a solution of a catalytic metallic halide in ethyl ether at a temperature favorable to polymerization of polymerizable constituents present in said motor fuel but insufficiently high to effect substantial 110 breaking down or cracking.

115 2. The process of stabilizing a petroleum distillate coming within the range covered by kerosene and lighter fractions, which comprises commingling such a distillate with a solution of aluminum chloride in ethyl ether.

120 3. The process of producing a stable motor fuel which comprises subjecting an unstable petroleum distillate having a specific gravity of between .730 and .780 to the action of a metallic halide having a polymerizing action on gum-forming constituents in said distillate, said metallic halide being dissolved in ethyl ether, and separating resultant gummy products from the liquid.

125 4. The process of producing a stabilized petroleum product which comprises subjecting a cracked petroleum distillate having a specific gravity of between .730 and .830 to the action of a metallic halide having a poly-

- merizing action on gum-forming constituents in said distillate, said metallic halide being dissolved in ethyl ether, and separating resultant gummy products from the liquid.
5. The process of producing a stable motor fuel which comprises subjecting a hydrocarbon motor fuel distillate to the action of a solution of a catalytic metallic halide in ethyl ether, the amount of said metallic halide used being less than one per cent of the distillate by weight, and separating resultant gummy products from the liquid.
6. The process defined in claim 5, in which separation of resultant gummy products is effected by re-distilling.
7. The process defined in claim 5, in which the catalytic metallic halide is anhydrous aluminum chloride, employed in amount equal to less than one per cent of the distillate by weight.
8. The process of producing a stable motor fuel which comprises subjecting a crude motor fuel containing up to about 40 per cent of unsaturates to the polymerizing action of less than 1 per cent of anhydrous aluminum chloride dissolved in ethyl ether, said motor fuel having been derived from petroleum oil by suitable heat treatment, and distilling a substantially stable motor fuel product from the crude motor fuel thus treated.
9. The process of modifying hydrocarbon oils which comprises subjecting a hydrocarbon oil under reacting conditions to the modifying action of a catalytic metallic halide dissolved in ethyl ether.
10. The process of modifying hydrocarbon oils containing polymerizable constituents which comprises subjecting such a hydrocarbon oil under reacting conditions to the action of a solution of aluminum chloride in ethyl ether.
11. The process of modifying hydrocarbon oils which comprises subjecting a hydrocarbon oil under reacting conditions to the modifying action of a catalytic metallic halide dissolved in an ether of the oxide type.
12. The process of modifying hydrocarbon oils which comprises subjecting a hydrocarbon oil under reacting conditions to the modifying action of aluminum chloride in an ether of the oxide type.
13. The process of producing a stable motor fuel which comprises subjecting a hydrocarbon motor fuel distillate to the action of a solution of a catalytic metallic halide in an ether of the oxide type, the amount of said ether used being less than one per cent of the distillate by weight, and separating resultant gummy products from the liquid.
14. The process of producing a stabilized petroleum product which comprises subjecting a cracked petroleum distillate having a specific gravity of between .730 and .830 to the action of a metallic halide having a poly-
- merizing action on gum-forming constituents in said distillate, said metallic halide being dissolved in an ether of the oxide type, and separating resultant gummy products from the liquid.
- In testimony whereof I hereunto affix my signature.
- WILLIAM G. LEAMON.
- 70
- 75
- 80
- 85
- 90
- 95
- 100
- 105
- 110
- 115
- 120
- 125
- 130